

## UNITED STATES PATENT OFFICE

2,429,089

## PRODUCTION OF ELECTRICAL CONDENSER PLATES

Ernest Robert Box, London, England, assignor to  
 Johnson, Matthey & Company Limited, London, England, a British company

No Drawing. Application September 14, 1944,  
 Serial No. 554,143. In Great Britain October  
 13, 1943

2 Claims. (Cl. 117—46)

1

In my prior application Serial No. 487,651, filed May 19, 1943, I have described a process for producing electrical condenser plates which consists in applying to a suitable dielectric by means of a meshed printing screen a paste comprising a mixture of an organic liquid screen-printing medium with a metal compound decomposable by heat to leave a residual metal film and thereafter firing at such a temperature and for such a period of time that the organic matter is burned away and the metal compound is decomposed to yield a layer of metal which adheres firmly to the dielectric.

I have now found that in the said process I can use, instead of a metal decomposable by heat, metallic silver provided the silver is in a finely divided form.

The process according to the present invention therefore consists in applying to a suitable dielectric by forcing through a stencil or the like affixed to a meshed printing screen by means of a roller or squeegee a paste comprising a mixture of an organic liquid screen-printing medium with finely divided metallic silver and thereafter firing at such a temperature and for such a period of time that the organic matter is burned away and the silver is left as a layer adhering firmly to the dielectric.

The silver is preferably brought into a finely divided form for use according to the present invention by a precipitation method.

For example the silver may be directly precipitated from a solution of a silver salt, such as silver nitrate, by the addition of an organic reducing agent, such as formic acid, or by the addition of an inorganic reducing agent, such as sodium hypophosphite.

The finely divided silver may also be obtained from a solution of a silver salt by displacement of the silver therefrom by adding to the solution an excess of another metal, such as zinc, which is preferably in finely divided form. The resulting powder, which consists of the whole of the silver from the silver compound together with the excess of the other metal, may then be freed from said other metal by treatment with an acid, such as dilute sulphuric acid, which will dissolve the other metal but which will have no effect on the silver.

Another method of preparing the finely divided silver is by the reduction of precipitated silver chloride by means of zinc powder and sulphuric acid.

Apart from the substitution of metallic silver for the metal compounds described in my said

5 prior specification Serial No. 487,651, the process is identical with the process described in the said application.

In the process, as now practised, the screen 10 consists of a piece of, for example, silk or other woven material stretched over a frame and the meshes of the screen are obscured by a stencil or by a suitable filler except at the parts where it is desired that the paste comprising the metallic silver and the liquid medium should pass through onto the dielectric. While the paste is usually applied to the dielectric in the shape of a rectangle or square, any other shape may be applied if desired. The paste is forced through the screen 15 for example by means of a roller or squeegee after the dielectric has been located in the appropriate position under the screen.

It is preferred to use mica as the dielectric, but any other dielectric which is suitable for condenser plates and which is capable of withstanding the firing operation may be used. Examples 20 of such other dielectrics are glass and porcelain.

The liquid screen-printing medium which is 25 used for making the powdered silver into a paste suitable for application to the dielectric by means of a screen should be relatively viscous so as to form a paste which can be squeezed cleanly through the mesh of the printing screen to give a continuous uniform layer of paste which when 30 subsequently heated leaves a residual metal film free from bubbles and cracks. Examples of such media are solutions of a cellulose ester or ether in a volatile organic ester solvent, or solutions of drying oils, gums, and synthetic and natural resins in appropriate volatile solvents. I have found 35 that very satisfactory results may be obtained with a solution of cellulose nitrate or ethyl cellulose in ethyl, amyl or butyl acetate, lactate or phthalate. In some cases it is advantageous to add to the liquid medium a plasticiser, such as diethyl or dibutyl phthalate, medicinal paraffin, 40 castor oil or methyl abietate.

45 Adherence of the metal film to the dielectric may be improved where desired by the addition to the paste of a suitable flux, such for example as lead silicate, lead borate or lead boro-silicate, or the corresponding bismuth compounds or mixtures of two or more of the aforesaid.

After the paste comprising the metallic silver, 50 with or without the addition of a flux, has been applied to the dielectric by means of a screen, the firing operation is carried out by heating at such a temperature, generally from 400° to 600° C., and for such a period, generally from 2 hours to 5

55 minutes (depending on the temperature), that

the organic matter is burned away, the metallic silver is converted into a metal film and this film adheres firmly to the dielectric.

The film of metal thus produced on the dielectric is of uniform thickness and texture throughout and the condenser plates obtained have excellent electrical properties.

The following example will further illustrate how the said invention may be carried out in practice, but the invention is not restricted to this example.

*Example*

A paste of a consistency suitable for application through a screen is made from finely powdered silver and an 8% solution of cellulose nitrate in butyl lactate. If desired, 3% of lead borosilicate, calculated on the weight of silver, may also be added as a flux to improve the adherence of the silver film later to be formed.

A strip of mica, cut to the appropriate size, is then located beneath a screen to which has been applied a stencil having an aperture of the exact area and shape of the film of silver which it is desired to apply to the mica. The paste prepared as above is then forced through the screen on to the mica by drawing a squeegee across the upper surface of the screen. The layer of paste is allowed to dry and then another layer is applied to the reverse side of the mica.

The mica bearing the two layers of paste is then fired at a temperature of 500° C. for 40 minutes.

This method of application, followed by the firing process as described, provides on each side of the plate a continuous compact film of silver of uniform thickness and texture. This film adheres firmly to the plate and all air between the mica and the silver is thereby excluded. Condenser plates produced as described in this example are characterised by high electrical capacity, non-variability of capacity under varying working conditions and minimum deviation of the

phase angle from 90° when used with alternating currents.

What I claim is:

1. A process of producing electrical condenser plates which consists in applying to mica by means of a meshed printing screen a paste made from finely divided metallic silver, a lead borosilicate flux and a solution of cellulose nitrate in butyl lactate and thereafter firing at 500° C. for 40 minutes.
2. A process of producing electrical condenser plates which consists in applying to mica through a meshed printing screen a paste made from finely divided metallic silver, a lead borosilicate flux and a solution of cellulose nitrate in a solvent selected from the group consisting of amyl lactate and butyl lactate, and thereafter firing at a temperature from about 400° C. to 600° C. for from about two hours to about five minutes, depending on the temperature, until the organic matter is burned away and the finely divided metallic silver is converted into a layer of silver free of bubbles and cracks and of uniform thickness and texture which adheres firmly to the mica.

25

30

35

40

40

ERNEST ROBERT BOX.

REFERENCES CITED

The following references are of record in the file of this patent:

UNITED STATES PATENTS

| Number    | Name    | Date          |
|-----------|---------|---------------|
| 1,300,394 | Hoffman | Apr. 15, 1919 |
| 1,922,387 | Muller  | Aug. 15, 1933 |
| 1,977,625 | Ernst   | Oct. 23, 1934 |
| 2,344,081 | Claude  | Mar. 14, 1944 |

FOREIGN PATENTS

| Country       | Date          |
|---------------|---------------|
| Great Britain | Mar. 22, 1934 |
| Great Britain | Nov. 26, 1937 |